

Nov. 8, 1949

A. J. MORWAY

2,487,260

EXTREME PRESSURE LUBRICANT

Filed April 3, 1947



Arnold J. Morway Inventor  
By J. P. Young Attorney

Patented Nov. 8, 1949

2,487,260

# UNITED STATES PATENT OFFICE

2,487,260

## EXTREME PRESSURE LUBRICANTS

Arnold J. Morway, Clark, N. J., assignor to Standard Oil Development Company, a corporation of Delaware

Application April 3, 1947, Serial No. 739,172

4 Claims. (Cl. 252—29)

1

This invention relates to extreme pressure lubricants, and in particular to extreme pressure lubricants such as greases containing carbon black as a grease-structure-imparting agent.

In the art of making lubricating greases, it is well known that the addition of certain oil-soluble compounds such as lead soaps and compounds comprising chlorine, sulfur, phosphorus and the like, improve the load-carrying capacity of the grease. Some of these compositions depend for their effect upon a strengthening of the lubricating film, whereas others depend upon a chemical reaction which takes place at elevated temperatures when metal parts come into contact as a result of lubricating film failure.

In a co-pending application, Serial No. 570,783, filed by the present applicant and John C. Zimmer jointly, dated December 30, 1944 (now abandoned), there is disclosed a grease composition comprising a mineral lubricating oil compounded with from 5% to 20% of a so-called structural carbon black, particularly an acetylene black, which gives to the oil a structural relationship characteristic of greases, as distinguished from a mere thickening which is characteristic of certain loaded oils such as oils containing graphite and the like.

As more fully discussed in said co-pending application, certain carbon blacks, especially acetylene blacks, have been found suitable for imparting the grease-like structure to the lubricant, and have been termed "structure blacks." These carbon blacks are characterized by an apparent reticulate structure, as observed under the high-power electron microscope. They are adapted to form colloidal gels in a variety of organic liquids. Such liquids may include those liquid petroleum distillates above the naphtha range, to which the structural carbon blacks impart a thickening effect quite similar to that of the grease-forming soaps, when the latter are compounded with mineral lubricating oils. The acetylene black and certain others, for example, those produced in the electric arc treatment of petroleum fractions, have this "structural" or oil absorbing property.

The structural characteristics whereby blacks

2

of the type mentioned above appear to form a colloidal or a grease structure, apparently are related in some manner not clearly understood, to the particle size of the carbon with its related surface area and oil absorption characteristics.

Acetylene blacks which have been found most suitable may, for example, have a pH rating of about 7, and may be of such average particle size as about 43 millimicrons diameter, having a surface area of about 7 acres per pound. The modified channel blacks which are also suitable, though less suitable than the acetylene blacks as structure forming materials, are commonly of a lower pH value. With smaller particle size, the blacks become increasingly difficult to disperse in oil and hence less practical to use. They are of more intense black color, and good for printing inks, paints, etc., but objectionable as grease ingredients because of these properties.

20 In the co-pending application mentioned above, the structural carbon was employed primarily for the setting up of a grease structure with a mineral oil, other extreme pressure chemical agents being added to impart the extreme pressure characteristics to the lubricant. It has now been found that the effectiveness of certain commonly used extreme pressure ingredients may be increased by a choice of suitable non-structural carbon blacks, i. e., those having less oil absorption capacity such as certain high modulus furnace blacks, e. g., one known commercially as "Statex 93," in addition to the structural blacks mentioned above, and to accomplish this is an object of my invention.

35 When materials such as sulfurized, chlorinated or phosphorized additives are incorporated in lubricants containing structure blacks, it appears that such additives are at least partly absorbed by the blacks. As a result, they do not impart their full load-carrying properties to the greases. 40 In addition, particularly in the lubrication of anti-friction roller bearings, it is not desirable to incorporate highly chemically reactive extreme pressure additives, because these may cause corrosion at high temperatures, or may hydrolyze under wet conditions to give corrosive products.

Notwithstanding the objection to the use of

chemically reactive extreme pressure additives in roller bearing lubricants, it is commonly required by bearing manufacturers that greases for anti-friction bearings have a fairly high extreme pressure load-carrying capacity. For example, the Timken Roller Bearing Company commonly requires that greases designed for use with its bearings have a 33 pound satisfactory load, which corresponds to 20,000 pounds per square inch load-carrying capacity, as measured by the Timken extreme pressure testing machine.

While greases of the type described in application Serial No. 570,783, mentioned hereinabove, embodying merely structure blacks and extreme pressure additives, have mild extreme pressure properties, they cannot pass the requirements just mentioned. Hence a further object of the present invention is to improve the load-bearing characteristics of structure black greases without increasing their corrosivity.

I have found that when a small amount of the structure black, whether acetylene black or other analogous black as used in the greases disclosed in the aforesaid co-pending application, is replaced with a non-structural carbon black, preferably of fairly large particle size, such as the high modulus furnace black referred to above, the load-bearing capacity of the grease is materially improved. Thus, when greases are prepared as described in the aforesaid co-pending application, and are further compounded with so-called mild or non-corrosive extreme pressure additives which are well known in the art, such greases are found capable of carrying only a 24 pound satisfactory load, when tested on the Timken machine. When a small amount of the structure black is replaced with less oil-absorptive black, the load-bearing capacity using the same extreme pressure additive, increases to 33 pounds

size of the structure black. Thus, a satisfactory black for the above purpose may be a high modulus furnace carbon black (HMF), such as a black sold by the Columbian Carbon Company as "Statex 93." This black has a pH value of about 10 and a surface area of about 4 to 6 acres per pound. The average particle size appears to be of the order of 50 to 80 millimicrons in diameter, the particles tending to the spherical or particulate form rather than the branched chain or reticulate form characteristic of acetylene black. These blacks are relatively easily dispersed in mineral oil since with the larger particle size, the black does not tend to agglomerate as readily as the smaller particle size blacks. The smaller particle size blacks are more acidic and one distinguishing characteristic of the non-structural black mentioned above is its high pH value, as compared with the ordinary channel blacks, the acetylene blacks being intermediate in this respect. Carbon blacks of high pH are desirable to the extent that they contribute to oxidation stability of the grease.

The following table indicates the load-carrying properties of various carbon black greases tested according to the present invention. The blacks such as those called "Monarch 80" were ordinary channel blacks, and the lubricating oils employed were refined mineral oils of 70 SSU viscosity at 210° F. It should be noted that grease containing only the channel blacks or acetylene blacks on the one hand, or containing only the less oil absorptive black such as the high modulus furnace black "Statex 93," on the other hand, were relatively unsatisfactory in certain respects, whereas a grease combining the two types of blacks passed the 33 pound test and even the 43 pound test without any difficulty.

TABLE I  
*Load-carrying properties of carbon black greases*

| Grease Composition                                                                                                                                                                                                                                                                                              | Load-Carrying Capacity as Measured by the Timken Extreme Pressure Testing Machine |         |         |         |                 |
|-----------------------------------------------------------------------------------------------------------------------------------------------------------------------------------------------------------------------------------------------------------------------------------------------------------------|-----------------------------------------------------------------------------------|---------|---------|---------|-----------------|
|                                                                                                                                                                                                                                                                                                                 | 8#                                                                                | 16#     | 24#     | 33#     | 43#             |
| 18.0% Ink black ("Monarch 80"), 81.0% Refined mineral oil, 70 SSU at 210° F., 1.0% Polyisobutylene solution. <sup>1</sup>                                                                                                                                                                                       | pass...                                                                           | fail... |         |         |                 |
| 18.0% Ink black ("Monarch 80"), 20.0% Pb oleate conc. (50-50 min. oil, conc.), 1.0% Polyisobutylene solution, 10.0% Sulfurized fatty oil (8.5% S.), 51.0% Refined min. oil, 20.0% High modulus furnace black (Statex 93), 1.0% Polyisobutylene solution, 79.0% Refined min. oil. (Does not make a good grease.) |                                                                                   | pass... | pass... | fail... |                 |
| 20.0% Acetylene black, 1.0% Polyisobutylene solution, 79.0% Refined min. oil                                                                                                                                                                                                                                    |                                                                                   | do...   | do...   | pass... | fail...         |
| 12.0% Acetylene black, 1.0% Polyisobutylene solution, 20.0% Pb oleate conc. in min. oil, 20.0% PbS, 65.0% Refined min. oil                                                                                                                                                                                      |                                                                                   |         |         | pass... | fail...         |
| 12.0% Acetylene black, 1.0% Polyisobutylene solution, 20.0% Pb oleate conc. in min. oil, 5.0% Lord oil sulfurized 20%, 62.0% Refined min. oil                                                                                                                                                                   |                                                                                   |         |         | do...   | do...           |
| 12.0% Acetylene black, 1.0% Polyisobutylene solution, 20.0% Pb oleate conc. in min. oil, 7.5% $S_2Cl_2$ treated lard oil (cutting oil base), 59.5% Refined min. oil                                                                                                                                             |                                                                                   |         |         | do...   | do...           |
| 12.0% Acetylene black, 1.0% Polyisobutylene solution, 20.0% Pb oleate conc. in min. oil, 7.5% Sulfurized fatty oil, 8.5% S., 59.5% Refined min. oil                                                                                                                                                             |                                                                                   |         |         | do...   | do...           |
| 10% Acetylene black, 6% High modulus furnace black (Statex 93), 20% Lead oleate conc. in min. oil, 1% Polyisobutylene solution, 7.5% Sulfurized fatty oil, 8.5% S., 55.5% Refined min. oil                                                                                                                      |                                                                                   |         |         | do...   | pass... pass... |

<sup>1</sup> 1% polyisobutylene solution is 1% by weight of a mineral oil solution containing 6% by weight of isobutylene polymer of 50,000 to 100,000 molecular weight. Actual polyisobutylene content is .06%.

and even up to 43 pounds or more satisfactory Timken load, thus rendering such greases suitable for the lubrication of Timken roller bearings without adding more potent but objectionably corrosive types of extreme pressure agents.

The less oil-absorptive black which is preferably employed is not greatly different in particle size from acetylene black, although the average ultimate particle size may be somewhat larger. It should not be more than about twice the particle

The mineral oils mentioned above were all of 70 SSU viscosity at 210° F. The polyisobutylene compound was added to increase the tackiness of the grease.

Inasmuch as greases of the foregoing character may be used under conditions where considerable heat develops, and also where water may gain access or where water may be released as a result of chemical reaction of special additives, tests were also made as to the effects of heat and water on

the greases. The following table shows the results of such tests:

TABLE II

| Lubricant                                                                                                                                                                                                                | Conditions of anti-friction bearing cup after contact with the wet grease for 24 hours at 340-345° F. |
|--------------------------------------------------------------------------------------------------------------------------------------------------------------------------------------------------------------------------|-------------------------------------------------------------------------------------------------------|
| 6.0% High modulus furnace black (Statex 93), 10.0% Acetylene black, 1.0% Polyisobutylene solution, 20.0% Pb oleate conc. in min. oil, 63.0% Refined coastal oil—70 SSU at 210° F., 33 1/4% water in contact with grease. | Unchanged, Like Original.                                                                             |
| Same grease base containing 2.0% chlorinated wax (40% chlorine—typical commercial extreme pressure additive for greases) in place of sulfurized fatty oil, 33 1/4% water in contact with grease.                         | Darkened and corroded.                                                                                |

An example of a suitable composition for a mild E. P. base oil suitable for use in greases of the foregoing character has been found to be as follows:

|             | Per cent |
|-------------|----------|
| Sperm oil   | 70.4     |
| Sulfur      | 9.6      |
| Mineral oil | 20.0     |

The sperm oil was heated to 380° F. and the sulfur added. The temperature was maintained at 380-385° F. for 90 minutes, and the mineral oil added at the end of that period. The temperature was then reduced to 200° F. as rapidly as possible to eliminate further sulfurization.

Sulfur analysis per cent=8.5.

A carbon black grease may be prepared according to the following formula:

|                                        | Per cent |
|----------------------------------------|----------|
| High modulus furnace black (Statex 93) | 6.0      |
| Acetylene black                        | 10.0     |
| Polyisobutylene solution               | 1.0      |
| Lead oleate                            | 10.0     |
| Sulfurized fatty oil                   | 10.0     |
| Mineral oil 70 SSU at 210° F.          | 63.0     |

The carbon blacks are charged to the kettle and approximately 1/3 of the oil added. The temperature may be raised, but since little or no thinning out of the grease occurs with a rise in temperature, no particular advantage is gained. Paddle speeds should not be too fast at first or the black which is very light and fluffy may be blown out of the kettle. When the black and oil starts to ball up, more oil is added, working out to a smooth grease. When all the oil is in and the resultant grease smooth, the lead oleate is heated to approximately 200° F. to facilitate handling and then is charged and worked into the mass. Some softening usually occurs when the lead oleate is added. If facilities for heating the lead oleate are not available, the temperature of the grease in the kettle may be raised to 200° F. and the lead oleate concentrate then added. The sulfurized fatty oil is then added and thoroughly incorporated into the grease. The polyisobutylene is added last. The product having a worked penetration of 340/360 mm/10 is then filtered through equipment similar to that used on calcium greases and packaged.

Greases of this type, having a heavier consistency than that described above, may be prepared by increasing the carbon black. I have noted that greases containing 20% or more of carbon black set back to relatively hard products, which readily break down on very slight working to their original consistency.

As indicated above, it is preferred that the carbon black be divided between a reticulate or chain-like structure black and a particulate black which does not unduly absorb oil or the extreme pressure additive therein. Preferably 1/2 to 1/2 of the carbon black will be of the latter

type, such as the high modulus furnace carbon black of the "Statex 93" type.

Tests show that the carbon black greases of my invention are much more consistent in viscosity and structure over a wide temperature range, than is the case with certain standard recognized high temperature greases. The attached drawing shows the temperature-pressure characteristics of a grease containing the mixture of particulate and reticulate blacks as compared with a typical soap thickened grease currently sold on the market for lubrication at elevated temperature.

While I have indicated that various percentages of various types of carbon blacks may be used in greases, it will be understood that the proportions may vary according to the load-carrying characteristics desired, consistency, viscosity of the lubricant, E. P. additives used, and other variables. Thus, the percentage of particulate carbon black, i. e., the black of relatively lower grease-structure properties, may vary from a very small fraction to as much as or more than the amount of acetylene or other highly absorptive black used. The latter black may vary from 3 to 20% by weight of the entire grease, and the less absorptive black may vary from 0.5 to 10% or more. Various additives, such as antioxidants, corrosion inhibitors and the like, may be incorporated, as will be understood by those skilled in the art. The total carbon black content will ordinarily run between 5 and 25% by weight, based on the total composition.

As indicated above, the oil soluble polymer such as a polyisobutylene, used to impart adhesive properties, is preferably added as a concentrated oil solution. A desirable additive is a 6% solution in mineral oil, from 0.1 to 3% of such solution being added, based on the total grease composition. The actual polymer content of the finished grease is therefore from 0.006 to 0.18%, a content of about 0.05% to 0.10% being preferred.

I claim:

1. A composition consisting essentially of

|                                                 | Per cent |
|-------------------------------------------------|----------|
| Acetylene black                                 | 10       |
| High modulus black                              | 6        |
| Lead oleate                                     | 10       |
| Oil solution of polymer for imparting tackiness | 1        |
| Sulfurized fatty oil                            | 10       |
| Refined mineral oil of lubricating grade        | 63       |

2. A composition substantially as given in claim 1 where the non-corrosive extreme pressure agent is sulfurized sperm oil.

3. An antifriction-bearing lubricant consisting essentially of a major proportion of lubricating oil, 5 to 25% carbon black including both a major proportion of acetylene and a minor proportion of high modulus carbon blacks, 2 to 15% lead oleate, 2 to 15% sulfurized fatty oil, and 0.05 to 0.10% of an oil soluble polymer capable of imparting adhesive properties to said composition,

said composition being non-corrosive to said bearings.

4. An extreme pressure lubricant comprising at least 60% mineral lubricating oil, 5 to 25% carbon black containing 3 to 20 parts of acetylene black and 0.5 to 10 parts of high modulus black, the acetylene black being always present in larger amount than said high modulus black and a metal soap, a tackiness agent, and a non-corrosive extreme pressure agent.

ARNOLD J. MORWAY.

REFERENCES CITED

The following references are of record in the file of this patent:

UNITED STATES PATENTS

| Number      | Name         | Date          |
|-------------|--------------|---------------|
| 2,179,063   | Smith et al. | Nov. 7, 1939  |
| 5 2,349,058 | Swenson      | May 16, 1944  |
| 2,356,367   | Wright       | Aug. 22, 1944 |

OTHER REFERENCES

10 Rubber Age, August 1944, article by Sweiitzer and Goodrich entitled "The Carbon Spectrum for the Rubber Compounds," page 470.

Can. Chem. & Process Ind., March 1944, article by Wiegand entitled "Recent Developments in Colloidal Carbon," page 160.